

*J. B. Crowley,*

*Metallic Roofing.*

*No. 95,990.*

*Patented Oct. 19, 1869.*

*Fig. 1.*



*Fig. 2.*



*Witnesses:*

*J. J. Libbey  
J. H. Thummay*

*Inventor:  
Job B. Crowley,*

*John E. Earle  
Attorney*

# United States Patent Office.

JOB B. CROWLEY, OF MIDDLETOWN, CONNECTICUT, ASSIGNOR TO HIMSELF  
AND MANNING, BOWMAN & CO., OF SAME PLACE.

*Letters Patent No. 95,990, dated October 19, 1869.*

## IMPROVED METALLIC ROOFING.

The Schedule referred to in these Letters Patent and making part of the same.

*To all whom it may concern:*

Be it known that I, JOB B. CROWLEY, of Middletown, in the county of Middlesex, and State of Connecticut, have invented a new Improvement in Enamelled Corrugated Roofing and I do hereby declare the following, when taken in connection with the accompanying drawings, to be a full, clear, and exact description of the same, and which said drawings constitute part of this specification, and represent, in—

Figure 1, a top view of a piece of roofing, and in Figure 2, a transverse section of the same.

This invention relates to an improvement in metal roofing, and is especially adapted to that commonly known as corrugated roofing, the object being to avoid the use of paint or similar coating, which wears away so as to require recoating; and

The invention consists in coating the metal, upon one or both sides, with porcelain-clay, or other vitreous material, while in a plastic state, then, by heat or otherwise, hardening the coating.

To enable others skilled in the art to make and use my invention, I will fully describe the same, as illustrated in the accompanying drawings.

By preference I form the metal in plates, as seen in fig. 1, the several plates corresponding in size, and corrugated as seen in section, fig. 2, each plate being perforated, as a means of securing to the roof.

Then I coat upon the upper side, (and, by preference, both sides,) by spreading thereon a coating of porcelain-clay, or other vitreous substance, while in a plastic state, and then harden the coating by subjecting it to the heat or a drying-process, and when hardened, the roofing is ready for use, to be applied in the usual manner of similar metal roofing.

This coating is not affected by the atmosphere, and is not in the slightest degree worn away, as other coating, or paint.

Having fully described my invention,

What I claim as new and useful, and desire to secure by Letters Patent, is—

As a new article of manufacture, metallic roofing, coated upon one or both sides, with porcelain, or other vitreous material, substantially as set forth.

JOB B. CROWLEY.

Witnesses:

J. H. SHUMWAY,  
A. J. TIBBITS.